

## UNITED STATES PATENT OFFICE

ORIN A. BASSETT, OF OKLAHOMA CITY, OKLAHOMA, ASSIGNOR TO THE NATIONAL INDUSTRIAL LABORATORIES CORPORATION, OF OKLAHOMA CITY, OKLAHOMA, A CORPORATION OF DELAWARE

## PROCESS FOR TREATING METALLIC ARTICLES

No Drawing.

Application filed November 6, 1925. Serial No. 67,453.

After iron or steel has been coated with a metal of lower melting point, it has heretofore been impossible to heat-treat the iron or steel without destroying the coating. Tin or 5 zinc coating on iron or steel has thus been narrowly confined to such articles as could be coated as a final step and so leave the coating undisturbed. Correspondingly the 10 advantage of a cheap anti-rust coating for steel has been very sharply limited.

In accordance with my invention, metals after being coated with other metals which are inherently fugitive by reason of relatively low melting point or ready oxidizability may 15 be heat-treated variously as desired without in any way damaging the coating. In some conditions, the character of the coating may in fact be improved.

To the accomplishment of the foregoing 20 and related ends, the invention, then, consists of the features hereinafter fully described, and particularly pointed out in the claims, the following description setting forth but a few of the various ways in which the principle of the invention may be used.

In applying my process, I may proceed for example as follows: the article to be treated, for instance steel, is coated with a relatively low melting metal such as zinc, by hot or by 30 cold galvanizing, and is then coated or covered by about  $\frac{1}{8}$  to  $\frac{1}{2}$  inch thick (depending upon the size of the article) with what for want of a better name (and without committing myself to any theory of 35 action) I may call a fixative agent, and which comprises preferably a composition of potassium cyanide or sodium cyanide about 30 per cent., borax about 20 per cent., soda ash or sodium carbonate about 20 per cent., powdered carbon preferably graphite about 20 per cent. This may be applied dry where convenient by warming the steel article and plunging it into the powder so that enough will adhere, or the material may be made up with an adhesive 40 binder such as glue water or the like and be spread on by a brush, trowel or other convenient means. The steel article is now heated up to the temperature necessary, and is quenched by water, oil or other means for the tempering desired, and on cleaning, the

zinc coating will not only be found intact, but capable of taking on a superior polish. Instead of tempering, the steel article can be annealed, or the heating can be employed for the purpose of bending or shaping the 55 article. The feature in any case being the possibility of subjecting the metal-coated article to high temperatures for desired heat-treating or shaping, temperatures which would normally be destructive to the metal 60 coating, but which in accordance with my process are successfully borne. In this manner tools, implements, cutlery, etc. can be galvanized or tinned and afterwards tempered. I can in fact make needles of tinned 65 or galvanized iron wire and temper them to any desired hardness.

The process is not confined to steel or to articles coated with zinc but metal articles generally, coated with tin, copper, brass, lead, etc. may be similarly successfully heat-treated without destroying the metal-coating. Thus, not only steel but other iron-base articles can be treated, for instance iron wire 70 may be galvanized and then treated in accordance with this process, the wire being coated with the fixative agent and then subjected to a cherry-red heat for a few minutes to several hours, depending upon the size of the wire and the properties desired, and then 75 finally plunged into cold water. The wire will be found to be very tenaciously anti-rust coated and capable of taking a fine polish. I am unable to say just what chemical change 80 occurs, but the coating instead of as usual being more or less readily separated from the iron, is as the result of this process, blended more tenaciously into the body of the metal. In this manner wire and cables can be readily 85 provided which will have the desired tensile strength, hardness and malleability and be thoroughly rust-resisting for fencing, suspension bridge work, rigging, etc.

I may also take tinned or galvanized sheet 90 iron barrels or barrel stock and coat with the fixative and heat, and thus secure improved rust-resisting and wearing barrels, cans, etc.

By coating thin iron plates with the fixative and heating, then welding a number of 95 the plates together, placing galvanized 100

plates on the outside, superior built-up plate metal for safes, armor plate, etc. may be produced.

Other modes of applying the principle of my invention may be employed instead of the one explained, changes being made as regards the method and means herein disclosed, provided the step or steps or means stated by any of the following claims or the equivalent of such stated step or steps or means be employed.

I therefore particularly point out and distinctly claim as my invention:—

1. A process of treating metal coated with a more fugitive metal, which comprises heating the coated metal in the presence of a fixative agent including the element carbon.
2. A process of treating metal coated with a more fugitive metal, which comprises heating the coated metal in the presence of a fixative agent including a cyanide.
3. A process of the character described, which comprises applying a fixative agent including the element carbon to an iron-base article coated with a fugitive metal, and then heating.
4. A process of the character described, which comprises applying a cyanide and free carbon to an iron-base article coated with a fugitive metal, and heating.
5. A process of the character described, which comprises heating in the presence of a cyanide and graphite an iron-base article coated with a fugitive metal.
6. A process of treating metal coated with a more fugitive metal, which comprises applying a cyanide to the coated metal, and then heating.
7. A process of treating metal coated with a more fugitive metal, which comprises applying a fixative agent including a cyanide, borax, sodium carbonate and carbon, to the coated metal, and then heating.
8. A process of treating metal coated with a more fugitive metal, which comprises applying a fixative agent including a cyanide, borax, sodium carbonate and graphite, to the coated metal, and then heating.
9. A process of treating an iron-base article coated with a fugitive metal, which comprises applying a fixative agent including a cyanide, borax, sodium carbonate and graphite, to the coated metal, heating, and tempering.

Signed by me this 2nd day of November, 1925.

ORIN A. BASSETT.